# EUROPEAN PATENT SPECIFICATION

(11) **EP 0 066 019 B1**
(45) Date of publication and mention of the grant of the patent: **19.06.1985**
(21) Application number: 81302453.6
(22) Date of filing: 03.06.1981
(51) Int. Cl.: C23C 10/34, C23C 10/48, C23C 10/52

(54) **Diffusion coating composition and method**
Zusammensetzung und Verfahren zur Diffusionsbeschichtung
Composition et procédé pour le revêtement par voie de diffusion

(43) Date of publication of application: 08.12.1982
(73) Proprietor: WALBAR METALS, INC., Peabody Massachusetts 01960 (US)
(72) Inventor: Rose, Bernard R., Ipswich Massachusetts 01938 (US); Willis, John K., Salem New Hampshire 03079 (US)
(74) Representative: Funge, Harry

## Description

The invention relates to the diffusion coating of superalloys, such as high-nickel and high-cobalt alloys, wherein a part to be treated is placed in a coating, powder pack.

It is already known that diffusion coating of metallic objects, for example nickel- and cobalt-based alloys, may be carried out by embedding the article to be coated in a powdered coating pack including:
(1) an inert filler,
(2) a vaporisable carrier ingredient, and
(3) powdered sources of metal materials to be diffused into the superalloy object.

The vaporisable carrier ingredient, usually a halide composition, acts as a flux in facilitating the initial reaction between aluminum and the alloy being treated, and also acts to accelerate the diffusion process by forming intermediate or transient compounds during the process. In general, the vaporisable carrier material has been a halide, for example a fluoride or chloride salt, such as ammonium chloride. This relatively diffusable material provides means for carrying the treating metal into the superalloy surfaces to be treated.

The metal powder, usually aluminum or chromium, is the active metal-treating agent on which the carrier material acts to facilitate diffusion of the metal into the article to be treated.

The inert filler acts primarily as a means to moderate the concentration and rate at which the carrier material and diffusing metal approach the metal article to be treated. It is also a manipulative expedient which provides the function of reducing the cost of material expended in carrying out the process. Cost of the material in a powder pack usually requires that the pack is to be used for a number of treating cycles. In such cases the pack is usually refurbished with the more readily depleted components before proceeding from one cycle to another.

Processes of this general type have been disclosed by Wachtell and Seelig in U.S. Patent 3,257,230 and by Puyear and Schley in U.S. Patent 3,079,276. The object of such processes is to provide a protective outer sheathing on engineering parts subjected to high temperatures and corrosive atmospheres; for example, the turbine blades in jet aircraft engines are subjected to such temperature and environment.

Some additional prior art includes packings which utilise C₀₂AIₛ (e.g. PWA 273, a material sold by Pratt & Whitney Division of United Technologies, Inc. and packings such as those described in a number of Patents including U.S. Patents 3,716,398; 3,594,219; 3,577,268; 3,810,782, 4,024,294; 4,041,196; 3,979,274; and many more such patents primarily classified in U.S. Classification 117 (old) and Class 427. There are many aspects of these diffusion processes for pack cementation coatings that it would be desirable to enhance. Some such aspects relate to the mechanical properties of the powder composition: for example, it would be very desirable for the used coating powder to be readily released from some of the very small apertures and channels that are encountered in the alloy parts being treated. Moreover, it is always desirable to improve the "hot corrosion" resistance of internal as well as external surfaces of the parts by subjecting them to treatments of the type being described.

As will be described below, the invention described herein is based on the surprising discovery of the value of certain cementatious coating powders.

It is an object of the present invention to provide a method of codeposition of aluminium and chromium diffusion coatings on articles formed of nickel-based superalloys, whereby the articles are packed in a coating powder from which AI and Cr may be derived and thermally treated while being packed in the coating powder in order to form a protective coating on said articles by the help of AI and Cr, characterised in that 1 to 15 wt% of the compound Co_{Z}Al₉ has been added to the coating powder.

It is a further object of the present invention to provide a method of codeposition of aluminium and chromium diffusion coatings on the internal surfaces of articles formed of nickel-based and cobalt-based super alloys whereby the articles are packed in a coating powder from which AI and Cr may be derived and thermally treated while being packed in the coating powder in order to form a protective coating on said internal surfaces of said articles by the help of AI and Cr, characterised in that 1 to 15 wt% of the compound C₀₂AIg has been added to the coating powder as the aluminium contributory chemical in said powder pack and Cr powder (passes 325 mesh) has been added to the coating powder as the chromium contributing chemical in said powder pack.

A more particular object of the invention is to provide a cementation powder composition, from which aluminium and chromium is expelled by thermally treating said powder composition and which is resistant to being immobilised by a heat treatment at about 1093° and remains readily flowable after two hours of such treatment comprising an inert filler, a halide carrier, chromium metal powder and an aluminium-contributing powder of the compound Co₂AIg in an amount of 1 to 15 wt%.

Another object of the invention is to provide compositions of superior flowability after they have been subjected in processing temperatures.

Other objects of the invention are to obtain an improved diffusion coating process, one which may be used to achieve more rapid processing and one which may be used to achieve superior properties of the processed goods.

Other objects of the invention will be obvious to those skilled in the art on their reading of this disclosure.

The above objects have been substantially unexpectedly and surprisingly achieved by the development and use of a powdered cementation pack coating composition comprising 1 to 15 wt % of the inter-metallic powder CO₂Al₉, particularly the powder which passes 325 mesh.

The amount of CO₂Al₉ that is utilised in the composition of the invention will differ somewhat depending on the particular use of the coating. For example, different quantities will be used in packings that are intended for internal surfaces (i.e. surfaces of interstices or orifices) and in external surfaces (i.e. the larger exterior surface of a part). One advantage of the compositions of the invention is the fact that they can readily be used in a single coating operation both for internal and external use. Another advantage is that the processes may be carried out at lower time-temperature profiles than processes carried out with such intermetallics as Co₂Alₛ, Cr₈Al₅ or CoAl.

The superalloys which are believed to be most advantageously treated by the process of the invention are the nickel-based superalloys especially e.g. those comprising about 16% chromium or less. Particular advantage is achieved with those alloys such as are known as IN100 and IN713 and IN792 which contain about 13% chromium or less.

It will be understood by those skilled in the pertinent art that the compositions of powder- pack compositions are varied depending upon the particular application involved. For example, somewhat higher chromium content in the metal being treated usually dictates a somewhat higher chromium content in the powder to facilitate diffusion of chromium into the surface of the metal. Likewise, the presence of cobalt in the metal shows diffusion of aluminium and this effect can be counteracted by changing the powder composition. Also, the powder weight to surface area ratio is so different for internal surfaces of a part being treated from powder weight to surface area ratio achieved by exterior surfaces, that this factor dictates substantial changes in coating powder composition. (Thus, for example, the internal surfaces of a part being prepared for treatment could suitably contain a coating powder composed of 8 to 10% Co₂Al₉ and 3 to 4% chrome, whereas the external surfaces being prepared for treatment might be packed with a mixture of 3-4% C₀₂AIg and 2-4% chrome.)

The process of the invention can typically be accomplished in less than half the time required for similar processing with conventionally used powder packings. For example, a cycle time of about 1 1/2 hours can be used in some applications as opposed to 3 to 4 hour cycles achieved with powder pack compositions which are presently available. Thus a 50 microns thich diffusion coating can be imparted to, say IN100 or IN713 alloy in 1 1/2 hours at a heat treating temperature of 1052°C, whereas the same result would take at least about twice as long using the powder packs of the prior art.

Oxidation resistance of coatings prepared according to the invention may be improved from 100% to 200% over coatings of the prior art, when utilising a 3% Co₂Alg, 2% chromium powder pack ("3-2 mix"). This has been shown by a high velocity oxidation test which is intended to be a partial simulation of operating conditions in the hot zone of a jet engine. Excellent results are also achieved with a 3-4 mix. Thus products comprising the diffusion coating of the invention exhibit excellent oxidation/ablation resistance at temperatures of 1093-1149°C.

A simulated Inconel 713 turbine blade coated with a co-deposited diffusion coating derived from a 3% C₀₂AIg 4% Cr pack, shows hot corrosion resistance approximately 50% greater than a "state of the art" aluminide coating. This has been validated by a 943°C-954°C hot corrosion test which, in part, simulates jet engine operating conditions.

One valuable and novel characteristic of the compositions of the invention is that they are resistant to being immobilized by a heat treatment in Argon at about 2000°F (1093°C) and, therefore, remain readily flowable after two hours of such a treatment.

In this application there is shown and described preferred embodiments of the invention and suggested various alternative and modifications thereof, but it is to be understood that these are not intended to be exhaustive and that other changes and modifications can be made within the scope of the invention. These suggestions herein are selected and included for purposes of illustration in order that others skilled in the art will more fully understand the invention and the principles thereof and will be able to modify it, each as may be best suited in the condition of a particular case.

### Example 1

A turbine blade, whose service condition has been categorized by a jet engine operator as high oxidation and cast from a high-nickel alloy sold under the trade designation "IN-100" by the International Nickel Company, was degreased by exposure to trichloroethane solvent vapours. (After this degreasing all handling of the turbine blade was carried out with cotton glooves). Thereupon the area of the turbine blade to be subjected to the diffusion coating process was abrasively cleaned with AI₂0₃ grit which had passed a 120 mesh sieve but has been retained on a 220 mesh sieve. After this blasting process, the turbine blade was once more degreased.

After these preparatory steps, the turbine blade was packed into a coating container, which has been prepared according to procedures known in the art and packed in a coating powder formulation comprising:

This is designated as the RB-505A blend for applications requiring high oxidation resistance. Workpieces should be placed in the coating container in such a way that there is about a 12.7 mm gap between adjacent pieces.

The powder box was loaded into a retort which is provided with means to circulate gas therethrough, means to insert thermocouples thereinto for the remote reading of temperature therein and a sand seal to prevent the ingress of air thereto. After the retort was closed, it was purged with Argon gas at a rate of about 7 volume changes per hour and then placed into a gas-fired pit furnace. Argon gas was constantly fed into the retort at a rate of about 5 volume changes per hour as the temperature inside the retort was rapidly raised to 1052°C and held there for an hour. The retort was then withdrawn from the furnance, and the parts were unpacked from the powder pack.

The coated nickel-base turbine blades were carefully cleaned with a stiff-bristled brush and compressed air. Thereupon, the part was inspected and washed for three minutes in warm water and dried.

The parts were then loaded in a clean retort not previously used for diffusion coating and heat treated in a hydrogen atmosphere for one hour at 1066°C. Purging technique and gas flow rates were similar to that described for the coating process, above.

After metallographic examination of a test piece so treated, an excellent codeposited diffusion coating of about 63.5 microns on depth was achieved during this process.

### Example 2

Example 1 was repeated but now a turbine nozzle guide vane of Inconel 738 alloy whose service condition has been categorised by a jet-engine operator as high hot corrosion. The following powder formulation was used:

This is designated as the RB505-B blend for applications requiring high hot corrosion resistance.

The pack temperature was 1066°C and the treatment time was two hours in an Argon atmosphere. The post-treatment was at 1079°C for one hour in a hydrogen atmosphere and resulted in an excellent codeposited diffusion coating of aluminum and chrome of 63.5 microns in depth.

### Example 3

This example relates to a hollow-turbine blade with internal cooling passages.

Example 1 was repeated excepting that the parts being treated had small apertures or conduits about 0.51 mm in diameter. The parts were supported on a vibrating table so that orifices, conduits and interstices, as small as 0.25 mm, were upwardly. Lower outlets of such orifices were taped to prevent egress of powder. Then, while the table vibrated, the orifices, conduits and interstices were filled with a powder of the following formulation:

This is designated as the RB505-C blend for applications requiring high hot corrosion resistance of internal surfaces.

After the interstices were filled and the upper outlets taped shut, vibrating was continued for about two minutes. Thereupon, the turbine blades were carefully packed in powder of the following formula, the RB505-B blend.

Thereupon, the heat treating step was carried out at about 1052°C for two hours in an argon atmosphere and an excellent codeposited diffusion coating was obtained simultaneously on the interior and exterior surfaces of the articles being treated.

## Claims

1. A method of codeposition of aluminium and chromium diffusion coatings on articles formed of nickel-based superalloys, whereby the articles are packed in a coating powder from which AI and Cr may be derived and thermally treated while being packed in the coating powder in order to form a protective coating on said articles by the help of Al and Cr, characterised in that 1 to 15 wt% of the compound Co₂AIg has been added to the coating powder.

2. A method as defined in Claim 1, characterised in that said article being treated is formed of a superalloy which comprises about 16% or less of chromium.

3. A method as defined in Claim 1, characterised in that said process is carried out on a superalloy comprising a maximum of about 14% chromium and within about two hours at a temperature of about 1052°C.

4. A method as defined in Claim 1, characterised in that the article to be processed contains internal surfaces and wherein the process comprises the steps of simultaneously treating said internal surfaces with a second powder pack composition comprising at least twice as much C₀₂AIg as does a first powder pack composition which is used to treat the external surfaces of said article.

5. A method of codeposition of aluminium and chromium diffusion coatings on the internal surfaces of articles formed of nickel-based and cobalt based super alloys whereby the articles are packed in a coating powder from which AI and Cr may be derived and thermally treated while being packed in the coating powder in order to form a protective coating on said internal surfaces of said articles by the help of AI and Cr, characterised in that 1 to 15 wt% of the compound Co₂AIg has been added to the coating powder as the aluminium contributory chemical in said powder pack and Cr powder (passes 325 mesh) has been added to the coating powder as the chromium contributing chemical in said powder pack.

6. A cementation powder composition, from which aluminium and chromium is expelled by thermally treating said powder composition and which is resistant to being immobilised by a heat treatment of about 1093° and remains readily flowable after two hours of such treatment comprising an inert filler, a halide carrier, chromium metal powder and an aluminium-contributing powder of the compound C₀₂AIg in an amount of 1 to 15 wt%

7. A composition as defined in Claim 6, characterised in that said halide carrier is NaF.

8. A composition as defined in Claim 6, characterised in that said halide carrier is NH₄F.

9. A composition as defined in Claims 6 or 7 characterised in that the composition comprises from 2 to 6 wt% of chromium.

## Revendications

1. Procedé de codéposition de revêtement de diffusion d'aluminium et de chrome sur des articles formés de super-alliages a base de nickel, suivant lequel les articles sont enveloppés dans une poudre de revêtement de laquelle l'amuminium et le chrome peuvent être issus et sont traités thermiquement tout en étant enveloppés dans la poudre de revêtement afin de former un revêtement de protection sur lesdits articles au moyen d'aluminium et de chrome, caractérisé en ce que 1 à 15% en poids du composé Co₂A1₉ a été ajouté à la poudre de revêtement.

2. Procédé suivant la revendication 1, caractérisé en ce ledit article traité est formé d'un super-alliage qui comprend environ 16% au moins de chrome.

3. Procédé suivant la revendication 1, caractérisé en ce que ledit traitement est effectué sur un super-alliage comprenant un maximum d'environ 14% de chrome et pendant environ 2 heures à une température d'environ 1052°C.

4. Procédé suivant la revendication 1, caractérisé en ce que l'article destiné à être traité contient des surfaces internes et suivant lequel le traitement comprend les étapes qui consistent à traiter simultanément lesdites surfaces internes avec un deuxième mélange d'enveloppe de poudre comprenant au moins deux fois plus de CO₂Al₉ qu'un premier mélange d'enveloppe de poudre qui est utilisé pour traiter les surfaces externes dudit article.

5. Procédé de codéposition de revêtement de diffusion d'aluminium et de chrome sur les surfaces internes d'articles formés de super-alliages à base de nickel et de cobalt suivant lequel les articles sont enveloppés dans une poudre de revêtement dans laquelle l'aluminium et le chrome peuvent être issus et sont traités thermiquement tout en étant enveloppés dans la poudre de revêtement afin de former un revêtement de protection sur lesdites surfaces internes desdits articles à l'aide d'aluminium et de chrome, caractérisé en ce que 1 a 15% en poids du composé CO₂Al₉ a été ajouté à la poudre de revêtements en tant que substance chimique contribuant à l'apport d'aluminium dans ladite enveloppe de poudre et en ce que de la poudre de chrome (passant à travers un tamis n°325) a été ajoutée à la poudre de revêtement en tant que substance chimique contribuant à l'apport de chrome dans ladite enveloppe de poudre.

6. Composition de poudre de cémentation, de laquelle l'aluminium et le chrome sont expulsés par traitement thermique de ladite composition de poudre et qui n'est pas susceptible d'être figée par un traitement thermique à environ 1093°C et reste susceptible de s'écouler aisément après 2 heures d'un tel traitement, comprenant une matière de remplissage inerte, un porteur d'halogène, de la poudre de chrome métallique et une poudre contribuant à l'apport d'aluminium du composé CO₂Al₉ suivant une quantité allant de 1 à 15% en poids.

7. Composition suivant la revendication 6, caractérisée en ce que ledit porteur d'halogène est NaF.

8. Composition suivant la revendication 6, caractérisée en ce que ledit porteur d'halogène est NH₄F.

9. Composition suivant la revendication 6 ou 7, caractérisée en ce que la composition comprend de 2 à 6% en poids de chrome.

## Patentansprüche

1. Verfahren zur gemeinsamen Ablagerung von Aluminiumund Chrom-Diffusionsüberzügen auf Artikeln aus Superlegierungen auf Nickelbasis, bei dem die Artikel in ein AI und Cr bereitstellendes Beschichtungspulver gepackt und währenddessen wärmebehandelt werden, um mittels AI und Cr einen Schutzüberzug auf den erwähnten Artikeln zu bilden, dadurch gekennzeichnet, daß das Beschichtungspulver die Verbindung CopAlg in einem Anteil von 1 bis 15 Gew.-% enthält.

2. Verfahren nach Anspruch 1, dadurch gekennzeichnet daß der erwähnte behandelte Artikel aus einer Superlegierung mit maximal ungefähr 16% Chrom besteht.

3. Verfahren nach Anspruch 1, dadurch gekennzeichnet, daß der erwähnte Prozeß bei einer Superlegierung mit maximal ungefähr 14% Chrom und innerhalb ungefähr zwei Stunden bei einer Temperatur von ungefähr 1052°C durchgeführt wird.

4. Verfahren nach Anspruch 1, dadurch gekennzeichnet, daß der zu behandelnde Artikel Innenflächen besitzt und bei dem der Prozeß die gleichzeitige Behandlung der erwähnten Innenflächen mit einer zweiten Einsatzpulvermischung umfasst, die zumindest doppelt soviel CO₂Al₉ enthält, wie die zur Behandlung der Außenflächen des erwähnten Artikels verwendete erste Einsatzpulvermischung.

5. Verfahren zur gemeinsamen Ablagerung von Aluminiumund Chrom-Diffusionsüberzügen an den Innenflächen von Artikeln aus Superlegierungen auf Nickelbasis und Kobaltbasis, bei dem die Artikel in ein AI und Cr bereitstellendes Beschichtungspulver gepackt und währenddessen wärmebehandelt werden, um einen Schutzüberzug an den erwähnten Innenflächen der erwähnten Artikel mittels AI und Cr zu bilden, dadurch gekennzeichnet, daß das Beschichtungspulver die Verbindung Co₂AIg in einem Anteil von 1 bis 15 Gew.-% als Aluminium liefernde Chemikalie des erwähnten Einstazpulvers und Cr-Pulver (Durchlauf bei Sieb-Nr.325) also Chrom liefernde Chemikalie in dem erwähnten Einsatzpulver enthält.

6. Zementierungs-Pulvermischung, aus der Aluminium und Chrom durch Wärmebehandlung der erwähnten Pulvermischung ausgetrieben werden und die beständig gegen Immobilisierung durch eine Wärmebehandlung bei ungefähr 1093° ist und nach entsprechender zweistündiger Behandlung gut fließfähig bleibt, umfassend einen inerten Füllstoff, ein Träger-Halogenid, Chrompulver und ein Aluminium lieferndes Pulver der Verbindung CO₂Al₉ in einem Anteil von 1 bis 15 Gew.-%.

7. Mischung nach Anspruch 6, dadurch gekennzeichnet, daß NaF das erwähnte Träger-Halogenid bildet.

8. Mischung nach Anspruch 6, dadurch gekennzeichnet, daß NH₄F das erwähnte Träger-Halogenid bildet.

9. Mischung nach Anspruch 6 oder 7, dadurch gekennzeichnet, daß die Mischung zwischen 2 und 6 Gew.-% Chrom enthält.
